

## 1

3,344,508

## PROCESS FOR PRODUCING CLADDED FUEL ELEMENTS

Jacques André Stohr, Bures-sur-Yvette, France, assignor to Commissariat à l'Energie Atomique, Paris, France  
No Drawing. Filed Jan. 20, 1964, Ser. No. 338,621  
Claims priority, application France, Feb. 20, 1963,  
925,479

2 Claims. (Cl. 29—420.5)

The present invention relates to co-extrusion and co-rolling processes which are employed in particular for the purpose of obtaining fuel elements in the form of round bars, tubes or plates.

The invention is more especially concerned, among the aforesaid processes, with those which permit the possibility of obtaining said fuel elements from composite billets or blooms in which the core of these latter constitutes the fuel proper whereas the outer portion thereof constitutes the cladding material, and which effect at the same time the formation of a metallurgical bond between the fuel and the can as well as the shaping of the round bar, tube or plate.

In the processes of the prior art, the co-extrusion or co-rolling operation was performed either directly on a composite billet or bloom or alternatively on a composite billet or bloom which was placed within a jacket, the function of which was to ensure that materials to be transformed were protected from the surrounding atmosphere.

The performance of these operations without jacketing is subject to the disadvantages which arise from absence of protection, for example the nitriding and corrosion effects which result in the case of zirconium or zirconium alloys. Moreover, the use of conventional protective jackets of steel increases the cost price of the operation to a considerable extent.

The object of the present invention is to make the said processes such that these latter meet the various practical requirements more effectively than has hitherto been achieved, especially insofar as they permit the possibility of overcoming the drawbacks mentioned above by ensuring that the shaping operation and provision of a metallurgical bond are carried into effect in the correct manner without calling either for protective jacketing, controlled-atmosphere preheating furnaces or complex apparatus for the purpose of welding or sealing jackets or blooms which had been necessary up to the present time.

The invention mainly consists—after having effected the metallurgical bond by diffusion between the fuel and the can by means of thermo-pneumatic or hydrostatic machine—in subjecting the product obtained to a plastic state deformation process such as rolling or extrusion, at a temperature which is compatible with the materials employed.

Apart from this main arrangement, the present invention further consists in certain other arrangements which are preferably employed at the same time and which are to be considered either separately or in combination, namely:

The metallurgical bond between the fuel and the can is ensured, after sealing of the fuel-can assembly by welding, by maintaining said assembly at a suitable temperature and pressure during the time which is necessary to obtain a diffusion bond between the constituent materials;

## 2

The aforesaid operation is carried out under hydrostatic pressure (water or oil, for example);

The aforesaid operation is carried out directly on the can-fuel assembly in a neutral gas atmosphere (argon, for example);

The aforesaid operation is carried out on said assembly which has been previously enclosed within a sealed casting (thin sheet of steel or copper, for example) which is closed in a vacuum or in an inert gas, and the atmosphere can in that case be any suitable gas.

The invention will in any case be more clearly understood by perusal of the complementary description and of the example which now follows below, said complementary description and said example being given solely by way of indication and not in any sense by way of implied limitation.

The process in accordance with the invention makes it possible to replace the conventional protective jackets (for example of steel) which are both of substantial thickness and costly by thin-walled casings (of steel or copper sheet, for example). A further economic advantage of the process is that its dispenses with the use of furnaces for pre-heating at high temperature in a controlled atmosphere as well as the use of apparatus for welding and sealing jackets. Moreover, the process in accordance with the invention transforms the operations involving co-extrusion or co-rolling in a jacket at high temperature into operations involving co-extrusion or co-rolling without jacket at moderate temperature.

In the case, for example, of zirconium or its alloys, the fuel-can assembly will be processed within a thermo-pneumatic machine and brought therein to a temperature of 750° to 950° C. at a pressure of at least 30 kilograms per square centimeter and will be maintained therein for a period of time which depends on the pressure and temperature adopted.

Uranium-zirconium fuel elements containing 2 to 8% by weight of uranium and clad with zircalloy have been metallurgically bonded under the following conditions: Temperature, 800° C.; pressure, 300 kgs./cm.<sup>2</sup>; time, 30 minutes; gas, neutral gas (argon, for example, or air).

The fuel elements were placed, in the case of air, within the protective boxes of copper or steel sheet of  $\frac{5}{10}$  mm. thickness.

It was possible to carry out the rolling of said fuel elements in the cold or warm state, that is to say within the range which is comprised between room temperature and 400° C., and within which no nitriding of the zirconium takes place, this result being achieved without the aid of any protective expedient. The elements thus rolled have shown no defect in the zone which was bonded by diffusion as a preliminary step.

It will be understood that the present invention is not limited in any respect either to the mode of application or to the example of execution which has been more especially contemplated but is intended, on the contrary, to include within its scope all alternative forms.

What I claim is:

1. A process for producing a fuel element comprised of a core section constituting the fuel proper and an outer protective cladding for said core section, said process comprising the following steps: (a) contacting a uranium-zirconium fuel mixture containing from about 2 to 8%

weight uranium with a cladding zircalloy to form a composite; (b) subjecting said composite to a temperature of approximately 800° C., at approximately 300 kgs./cm.<sup>2</sup> pressure for a time of approximately 30 minutes in an inert atmosphere to thereby obtain a metallurgically bonded metallic material; and (c) subjecting the material obtained from step (b) to a plastic state deformation process at a temperature range of from room temperature to 400° C.

2. A process according to claim 1, wherein prior to step (b), the composite is enclosed and sealed in an evacuated casing comprised of metal sheeting having a thickness of approximately  $\frac{5}{10}$  mm.

## References Cited

## UNITED STATES PATENTS

|   |           |        |                       |            |
|---|-----------|--------|-----------------------|------------|
| 5 | 3,025,592 | 3/1962 | Fischer et al. -----  | 29—498 X   |
|   | 3,118,221 | 1/1964 | Turovlim et al. ----- | 29—420.5   |
|   | 3,194,643 | 7/1965 | Ma et al. -----       | 29—470.1 X |
|   | 3,235,958 | 2/1966 | Gauthron -----        | 75—214     |
|   | 3,243,871 | 4/1966 | Saur -----            | 29—155.5   |

10 JOHN F. CAMPBELL, *Primary Examiner.*

CHARLIE MOON, *Examiner.*

P. M. COHEN, *Assistant Examiner.*